

Feb. 15, 1938.

P. CYKAJLO

2,108,528

PROCESS OF UNITING METALS

Filed Sept. 26, 1935

Fig. 1



Fig. 2



Fig. 3



Fig. 4



Fig. 5



Fig. 6



Fig. 7



Fig. 8



PETER CYKAJLO  
INVENTOR

By Freeman, Sweet, Albrecht and Weidman  
ATTORNEYS

## UNITED STATES PATENT OFFICE

2,108,528

## PROCESS OF UNITING METALS

Peter Cykajlo, Mansfield, Ohio, assignor of one-half to Henry L. Goemann, Mansfield, Ohio

Application September 26, 1935, Serial No. 42,302

10 Claims. (Cl. 29—189)

This invention relates to the art of uniting metals, and has for an object the provision of a new and improved process of uniting metals, such as steel and copper, and a new and improved composite metal resulting from the practice of such process.

In the drawing accompanying this specification, and forming a part of this application, I have shown for purposes of illustration, certain 10 embodiments which my invention may assume, and in this drawing:

Figure 1 is a perspective view showing a cast tube of one of the metals which is to be united to another.

Figure 2 is a vertical sectional view of a water-cooled mold, in which the tube shown in Figure 1 is placed.

Figure 3 is a fragmentary perspective view of the mold containing the tube, and disclosing the manner in which molten metal is introduced into 20 the tube.

Figure 4 is a fragmentary, diagrammatic view of the manner in which the united metals are treated after being removed from the mold.

Figure 5 is an enlarged sectional view through 25 the united metals following the treatment disclosed in Figure 4.

Figure 6 is a fragmentary perspective view of the united metals in sheet form.

Figure 7 is a fragmentary sectional view 30 through the sheet shown in Figure 6, such view corresponding substantially to the line 7—7 of Figure 6, while

Figure 8 is a fragmentary perspective view of 35 an expedient employed in connection with a different embodiment of the invention.

In carrying out the process, a tube of copper such as that shown at 10 of Figure 1, is first cast in a suitable mold. After the tube 10 has been 40 removed from the mold, the interior surface thereof is thoroughly cleaned through the application thereto of carbolic acid, or the like, and the tube 10 is then placed in an air-tight furnace and its temperature raised to between 1400° and 1800° Fahrenheit.

The heated tube 10 is then removed from the furnace and placed in a water-cooled mold, indicated at 11, in Figure 2, after which the interior of the tube 10 is sprayed with a flux mixture, 50 preferably comprising welding borax, calcium carbonate, ammonium chloride, and iron filings, in substantially equal proportions, and including glass dust, or fused silica, in a quantity about four times as great as the quantity of any one of the other described ingredients.

Low carbon low melting point steel is then heated separately, and in its molten state is poured into the tube 10, while the latter is in the mold 11, a ladle 12 being shown in Figure 3 in the act of pouring the molten steel into the 5 tube 10.

After the combined metals have been cooled sufficiently to be removed from the mold, the composite block 13 thus produced is then reheated to between 1800° Fahrenheit and 1900° Fahrenheit, 10 and subsequently rolled between sets of rolls 14 and 15 as shown in Figure 4.

Immediately prior to entering between the first set of rolls 14, however, the block 13 of reheated 15 united metals is sprayed with water on all exterior side and end surfaces, through the medium of high pressure jets 16, the spraying action continuing as the metals are slowly conveyed to a position to enter between the rolls 14.

The reheating and spraying just before rolling 20 comprise important features of applicant's invention, since reheating to the temperatures described causes the united metals to approach melted condition, while the spraying operation at high pressure hardens the exterior surfaces of 25 the block 13, and substantially seals the steel core therewithin, and causes the copper to contract upon the highly heated steel core. When entering between the rolls, the engaging surfaces of 30 the united metals being close to their melting 35 points, the contracting effect of the relative cold exterior of the copper tube, and the compressing action of the rolls, causes intercalation of the particles of the two metals, and thus provides a permanent union therebetween.

The resulting product is a rolled sheet 17 having 40 an exterior layer of copper 18 permanently united to the core of steel 19, and along the area of union the two metals exhibit a structure such as indicated at 20, in Figure 5, wherein the particles of the inner surface of the copper tube and the exterior surfaces of the steel core are intercalated to provide a permanent union.

In another embodiment of the invention, 45 wherein high melting point steel is employed, it is desirable to practice the process in this manner. An ingot of steel, illustrated at 21, in Figure 8, is first cast, and the ingot is then raised to or maintained at a temperature of from 1900° 50 Fahrenheit to 2000° Fahrenheit. After reheating the ingot, it is sprayed with a flux mixture such as that already referred to, and then set into a mold 22. Molten copper is then poured into the mold 22 so as to surround the steel ingot or core 21, and after the combined metals are removed 55

from the mold, they are reheated to a temperature of from 1700° Fahrenheit to 1900° Fahrenheit, and then sprayed and rolled in the manner heretofore described.

5. It will be understood to those skilled in the art that the process and resulting product embody at least the principal object of my invention, and concurrently, it also will be apparent that my invention has uses and advantages other than 10 those herein specifically mentioned; furthermore, it also will be appreciated that various changes and modifications may be made, without departing from the spirit of the invention; and accordingly, that the embodiments herein disclosed are 15 illustrative only, and that the invention is not limited thereto.

I claim:

1. A process for uniting metals, comprising: heating a plurality of metals, while juxtaposed, to 20 a temperature approaching the melting points thereof; exteriorly chilling said metals; and rolling said metals before the contacting surfaces thereof have cooled.

2. A process for uniting metals, comprising: 25 forming a metallic envelope of one metal and substantially enclosing another metal therewithin; heating the said metals while juxtaposed; exteriorly chilling said envelope to cause sealing of said envelope, and contraction of said envelope 30 upon the metal therewithin; and rolling said envelope and the metal enclosed therewithin before the contacting surfaces thereof have cooled.

3. The process for uniting metals, comprising: 35 forming a metallic envelope of one metal and substantially enclosing another metal therewithin; heating the said metals while juxtaposed to a temperature approaching the melting points thereof; exteriorly chilling said envelope; and rolling said envelope and the enclosed metal before the contacting surfaces thereof have cooled.

4. The process of uniting metals, comprising: 40 forming a metallic envelope and enclosing another metal therewithin; heating the said metals while juxtaposed to a welding temperature; directing jets of liquid onto the exterior of said envelope to chill the same; and rolling said envelope and enclosed metal while the contacting surfaces thereof are still at welding temperature.

5. The process of uniting metals, comprising: 5 forming a metallic envelope of one metal substantially enclosing the other metal by casting one of said metals about the other; reheating the said metals after casting to a welding temperature; exteriorly chilling said envelope; and rolling said envelope, with its enclosed metal, while the contacting surfaces thereof are still at welding temperature.

6. The process of uniting metals, comprising: 10 casting molten metal in contact with a solid metal; reheating the said metals after the casting operation to a temperature approaching the melting points thereof; exteriorly chilling said metals; and rolling said metals before the contacting surfaces thereof have cooled.

7. The process of uniting metals, comprising: 15 forming a metallic envelope of one metal substantially enclosing another metal by a casting operation; reheating the said metals after the casting operation to a temperature approaching the melting points thereof; exteriorly chilling said envelope; and rolling said envelope with its enclosed metal before the contacting surfaces thereof have cooled.

8. A process for uniting metals, comprising: 20 heating two different metals, while juxtaposed, to a temperature approaching the melting points thereof; exteriorly chilling said metals; and rolling said metals before the contacting portions thereof have cooled.

9. The process of uniting metals, comprising: 25 casting copper and steel to form an envelope of copper surrounding a core of steel; reheating the said metals after the casting operation; exteriorly 30 chilling said copper envelope; and rolling said copper envelope with its enclosed steel core before the contacting portions thereof have cooled.

10. A process for uniting unlike metals, comprising: 35 heating said metals while juxtaposed to a welding temperature; exteriorly chilling the outer surfaces of said metals, and rolling said metals while the contacting surfaces thereof are still at welding temperatures.

PETER CYKAJLO.